

# UNITED STATES PATENT OFFICE.

CHARLES R. SMITH, OF NEENAH, WISCONSIN.

## WATERPROOFING MATERIAL.

SPECIFICATION forming part of Letters Patent No. 607,773, dated July 19, 1898.

Application filed September 9, 1896. Serial No. 605,325. (No specimens.)

*To all whom it may concern:*

Be it known that I, CHARLES R. SMITH, a resident of Neenah, in the county of Winnebago and State of Wisconsin, have invented 5 certain new and useful Improvements in Waterproofing Materials; and I do hereby declare the following to be a full, clear, and exact description of the invention, such as will enable others skilled in the art to which it 10 appertains to make and use the same.

My invention relates to an improvement in waterproofing material, the object of the invention being to provide materials for waterproofing fiber and other material which shall 15 reduce the cost of such treatment to a minimum and at the same time result in a waterproof coating which shall possess adequate tenacity and power of penetrating the fiber and which will act to effectually exclude all 20 moisture from the fiber.

I first prepare a compound consisting of corn-oil and a gummy or resinous material, preferably rosin, in about the proportions of 25 seventy per cent. of corn-oil to thirty per cent. of rosin. By the term "gummy" it is intended to include only substances commonly used for varnishes, which, though technically resins, are known in the trade as "gums." The corn-oil will first be heated to a temperature 30 sufficient to drive out all moisture, (preferably about 500° Fahrenheit,) and then the rosin will be added. The compound thus made is not in any degree dangerous, as it is not inflammable, the use of naphtha or similar liquid heretofore employed being dispensed with.

When the temperature of the compound shall have diminished to about 350° Fahrenheit, (more or less,) the article to be treated 40 for waterproofing it will be immersed in the compound and allowed to remain therein a length of time sufficient to absorb an amount of the compound equal to about one-fourth its own weight. The article will then be removed and dried or baked, after which the 45 surface coating will be smoothed by sanding or in any other preferred manner. The ar-

ticle will then be dipped into a finishing compound consisting of corn-oil, linseed-oil, and rosin or other gummy or resinous material, 50 the oil having been first boiled, so as to thicken it, before the rosin is added, whereby the finishing compound will be of such consistency that an adequate coating can be applied to the article with a minimum number of applications. For treating ordinary pulp pails the finishing compound may consist of seventy-five parts of corn-oil, seventy-five parts of linseed-oil, and fifty parts of rosin. For 55 waterproofing some other articles the proportions may be varied more or less to advantage. When a more elastic or pliable coating is desired, the proportion of oil in both compounds will be increased and that of rosin diminished. When a harder coating is desired, a larger proportion of rosin and a smaller 60 proportion of oil than those above specified will be used.

After the article shall have been subjected to the finishing compound it will be again 65 dried or baked. If desired, the article may be several times subjected to the finishing compound and dried or baked after each application of the compound.

Extensive experiment has demonstrated 70 the value of corn-oil for waterproofing. It is very penetrating. Its cost is small and is effectual in the performance of its functions.

Having fully described my invention, what I claim as new, and desire to secure by Letters 75 Patent, is—

1. A waterproofing material consisting of corn-oil and a gummy or resinous substance, substantially as set forth.

2. A waterproofing compound consisting of 80 corn-oil, linseed-oil and a gummy or resinous substance, substantially as set forth.

In testimony whereof I have signed this specification in the presence of two subscribing witnesses.

CHARLES R. SMITH.

Witnesses:

H. J. MAYER,  
W. H. MINER.